# EUROPEAN PATENT SPECIFICATION

(11) **EP 4 122 363 B1**
(45) Date of publication and mention of the grant of the patent: **08.11.2023**
(21) Application number: 22181242.3
(22) Date of filing: 27.06.2022
(51) Int. Cl.: A47K 3/40, B32B 27/00

(54) **ULTRA-LIGHT SHOWER TRAY**
ULTRALEICHTE DUSCHWANNE
BAC DE DOUCHE ULTRA LÉGER

(30) Priority: 22.07.2021 ES 202131531 U
(43) Date of publication of application: 25.01.2023
(73) Proprietor: Mundo Gaman S.L., 28400 Collado Villalba (ES)
(72) Inventor: DÍAZ BLASCO, Enrique, 28400 Collado Villalba (ES); DÍAZ GRANDE, Sara, 28400 Collado Villalba (ES)
(74) Representative: Rodriguez Oca, Jesus

(56) References cited:
- DE-A1-102015 108 357
- DE-U1- 29 824 513
- GB-A- 2 402 363

## Description

The present invention relates to an ultra-ligh shower tray, thus finding its application in the field of manufacturing sanitary sanitations.

The shower tray of the invention, being very light, with a weight of approximately 12 kg/m², mineral-load trays weighing 45 kg/m2, offers numerous advantages in terms of installation and handling, while maintaining better performance in terms of mechanical stability, durability, installation and logistics.

Porcelain, acrylic, fiberglass-reinforced acrylic or mineral-filled resin shower trays are well known.

Known acrylic shower trays are made of an acrylic resin reinforced with fibreglass on the underside, their main disadvantage being the feeling of flexibility they give to the user, their poor mechanical stability and the difficulty of cleaning them, mainly due to the damage it can cause to the acrylic material. As for porcelain or mineral resin plates, they have the great disadvantage of their weight. GB-A-2.402.363 discloses an ultra-lightweight shower tray (10) comprising corresponding slopes towards a drain hole and a drain valve housing, wherein the tray (10) is made of a material composed of the following layers, indicated in successive order and taking the visible part of the shower tray as the top layer: a coating layer (11) based on an unsaturated polyester resin; a combined glass fibre layer of non-woven glass fibres wetted with an unsaturated polyester resin, a third layer and a fourth layer.

The present invention solves the disadvantages of known shower trays by providing an ultra-light shower tray with high mechanical stability, consisting of different layers of various materials, as will be described below.

The invention is now described in more detail on the basis of an example embodiment thereof and with reference to the attached figures, wherein:
Figure 1: Schematic plan view of the shower tray according to an example embodiment thereof;
Figure 2: Sectional detail of the drain valve housing of shower tray in figure 1;
Figure 3: Outline of the layered structure forming shower tray in figure 1; and
Figure 4: Shows a perspective view of drain valve housing in figure 2 and a detail thereof.

Figure 1 shows a schematic view of the ultralight shower tray of the invention (1), including corresponding slopes (2) towards a drain hole (3) and a drain valve housing (4), the detail of said housing (4) being shown in figure 2.

Referring now to figure 3, ultra-lightweight shower tray (1) consists of a material composed of the following layers, indicated in successive order and taking the visible part of shower tray as the top layer:
i. A coating layer based on an unsaturated polyester resin of isophthalic acid and neopentylglycol (5), with a thickness of 500 µm;
ii. A combined glass fibre layer of woven and non-woven glass fibres wetted with an unsaturated orthophthalic polyester resin (6), with a thickness of 3 mm;
iii. A layer of extruded polystyrene (7) pre-milled with shower tray slopes (2), with a thickness of 23 mm; and
iv. A layer of mesh-reinforced extruded polystyrene sheet coating mortar (8), with a thickness of 4 mm

In this figure 3, the different thicknesses of the layers that make up the shower tray are not scaled for better visualisation.

Drain valve housing (4) is arranged integrally with the shower tray embedded in layers i) and ii) described above and, as shown in figure 4, it is intended to receive a drain closure element (not shown), which may be a conventional grid or a cover made of the same material as described layer i), in this case in order to give the shower tray of the invention an homogeneous aesthetic finish. To this end, this drain valve housing (4) has corresponding internal support means (9) to support the aforementioned closure elements.

## Claims

1. An ultra-lightweight shower tray (1) comprising corresponding slopes (2) towards a drain hole (3) and a drain valve housing (4), wherein the tray (1) is made of a material composed of the following layers, indicated in successive order and taking the visible part of the shower tray as the top layer:
i. A coating layer based on an unsaturated polyester resin of isophthalic acid and neopentylglycol (5), with a thickness of 500 µm;
ii. A combined glass fibre layer of woven and non-woven glass fibres wetted with an unsaturated orthophthalic unsaturated polyester resin (6), with a thickness of 3 mm;
iii. A layer of extruded polystyrene (7) pre-milled with shower tray slopes (2), with a thickness of 23 mm; and
iv. A layer of mesh-reinforced extruded polystyrene sheet lining mortar (8), with a thickness of 4 mm.

2. An ultra-lightweight shower tray (1) according to claim 1, wherein the drain valve housing (4) is arranged integrally with the shower tray embedded in layers i) and ii).

3. An ultra-light shower tray (1) according to claim 1, wherein the drain valve housing (4) has corresponding internal support means (9) to support elements for closing drain hole (3).

4. An ultra-lightweight shower tray (1) according to claim 4, wherein closure elements of drain hole (3) are selected from a conventional grid or a cover made of the same material as layer i).

## Patentansprüche

1. Ultraleichte Duschwanne (1), die ein entsprechendes Gefälle (2) zu einem Ablaufloch (3) und ein Ablaufventilgehäuse (4) aufweist, wobei die Wanne aus einem Material besteht, das aus den folgenden Schichten besteht, die in aufeinanderfolgender Reihenfolge angegeben sind und wobei der sichtbare Teil der Duschwanne die oberste Schicht ist:
i. einer Deckschicht auf Basis eines ungesättigten Polyesterharzes aus Isophthalsäure und Neopentylglykol (5) mit einer Dicke von 500 µ;
ii. einer kombinierte Glasfaserschicht aus gewebten und nicht gewebten Glasfasern, befeuchtet mit einem ungesättigten orthophthalischen Polyesterharz (6), mit einer Dicke von 3 mm;
iii. einer Schicht aus extrudiertem Polystyrol (7), die zuvor mit dem Gefälle der Duschwanne (2) gefräst wurde, mit einer Dicke von 23 mm; und
iv. einer Mörtelschicht zur Verkleidung von Platten aus netzverstärktem extrudiertem Polystyrol (8) mit einer Dicke von 4 mm.

2. Ultraleichte Duschwanne (1) nach Anspruch 1, wobei das Ablaufventilgehäuse (4) einstückig mit der in die Schichten i) und ii) eingebetteten Duschwanne angeordnet ist.

3. Ultraleichte Duschwanne (1) nach Anspruch 1, wobei das Ablaufventilgehäuse (4) entsprechende innere Haltemittel (9) zum Halten von Verschlusselementen des Ablauflochs (3) aufweist.

4. Ultraleichte Duschwanne (1) nach Anspruch 3, wobei die Verschlusselemente des Ablauflochs (3) aus einem herkömmlichen Rost oder einer Abdeckung aus dem gleichen Material wie Schicht i) ausgewählt sind.

## Revendications

1. Receveur de douche ultraléger (1) qui comprend des baisses (2) correspondantes vers un trou (3) de vidange et un boîtier de vanne de vidange (4), dans lequel le receveur est constitué d'un matériau composé des couches suivantes, indiqués dans l'ordre successif et en prenant comme couche supérieure la partie visible du receveur de douche :
i. Couche de revêtement à base d'une résine polyester insaturée d'acide isophtalique et de néopentylglycol (5), avec une épaisseur de 500 µ ;
ii. Une couche de fibre de verre combinée de fibres de verre tissées et non tissées humidifiées avec une résine polyester orthophtalique insaturée (6), avec une épaisseur de 3 mm ;
iii. Une couche de polystyrène extrudé (7) préalablement fraisée avec les baisses du receveur de douche (2), avec une épaisseur de 23 mm ; et
iv. Une couche de mortier pour revêtir des plaques de polystyrène extrudé renforcé par maille (8), avec une épaisseur de 4 mm.

2. Receveur de douche ultraléger (1) selon la revendication 1, dans lequel le boîtier de vanne de vidange (4) est disposé d'un seul tenant avec le receveur de douche encastré dans les couches i) et ii).

3. Receveur de douche ultraléger (1) selon la revendication 1, dans lequel le boîtier de vanne de vidange (4) comporte des moyens de support internes (9) correspondants pour supporter les éléments de fermeture du trou de vidange (3).

4. Receveur de douche ultraléger (1) selon la revendication 3, dans lequel les éléments de fermeture du trou de vidange (3) sont choisis parmi une grille conventionnelle ou un couvercle réalisé dans le même matériau que la couche i).
